

## UNITED STATES PATENT OFFICE

GEORGE HOLLAND ELLIS, HENRY CHARLES OLPIN, AND ERIC EATON WALKER, OF SPONDON, NEAR DERBY, ENGLAND, ASSIGNORS TO CELANESE CORPORATION OF AMERICA, A CORPORATION OF DELAWARE

## COLORATION OF CELLULOSE DERIVATIVES

No Drawing. Application filed January 3, 1929, Serial No. 330,136, and in Great Britain January 30, 1928.

This invention relates to the dyeing, printing, stencilling or otherwise coloring of yarns, threads, woven or knitted fabrics or other materials made with or containing cellulose acetate or other organic esters of cellulose, for example cellulose formate, propionate or butyrate or the products obtained by the treatment of alkalinized cellulose with esterifying agents (e. g. the product known as "immunized cotton" obtained with p-toluene sulphonchloride), or made with or containing cellulose ethers, for instance methyl, ethyl or benzyl cellulose or the condensation products of cellulose and glycols or other polyhydric alcohols, all of which cellulose derivatives are hereinafter referred to as organic substitution derivatives of cellulose.

In the production of ice-colors upon cotton or other cellulosic fibres, such as the cellulosic type of artificial silk, the hydroxynaphthoic acid arylides have met with wide commercial application, the arylides being applied in the form of a solution of the alkali metal salts. In the production of ice-colors upon cellulose acetate or other cellulose ester materials three methods are available (a) application of the amine followed by diazotization on the fibre or material and treatment with a developer, (b) application of the developer component (e. g. phenolic compound) followed by development with a diazo solution and (c) application of amine and developer together or separately and subsequent diazotization on the fibre or material.

In methods (b) and (c), i. e. when the developer component is applied before any diazotization has taken place, it is essential in order to obtain good colorations that the developer component should be capable of being absorbed substantively by the fibre. It is found that this is not possible with the usual solutions of the alkali salts of hydroxynaphthoic acid arylides. If the impregnation be entirely mechanical the color formation is almost entirely superficial owing to this lack of absorption, so that the color rubs off badly and is also fugitive to washing, etc. If rinsing follows the impregnation with the alkali salt of the arylide before development

in the diazonium liquor, the arylide compound is largely removed.

We have discovered that these difficulties may be surmounted and useful colorations free from the above mentioned defects achieved by applying the hydroxynaphthoic acid arylides in the free state in a suitable dispersion. The absorption is such that there is even considerable resistance to intermediate rinsing.

We have further found that cellulose ether materials may likewise be successfully colored by applying dispersions of the free hydroxynaphthoic acid arylides.

Accordingly the present invention comprises processes for dyeing or otherwise coloring materials made with or containing cellulose acetate or other organic substitution derivatives of cellulose by applying dispersions of one or more free hydroxynaphthoic acid arylides either alone or together with a diazotizable amine and subsequently developing with a diazo-body or diazotizing on the fibre or material.

The dispersions of the hydroxynaphthoic acid arylides may be obtained by any suitable method, for example by fine milling or grinding (so-called "colloid milling") if desirable with the aid of dispersors and/or protective colloids; by dissolving in a solvent and mixing with water containing or not containing protective colloids or dispersors, e. g. soaps; or by treating the arylides with dispersors, for example as described in prior U. S. Patents Nos. 1,618,413, 1,618,414, 1,690,481, 1,694,413 and 1,716,721 and U. S. applications 1,694,413, 1,690,481, 152,517 filed 3rd December 1926, 134,138 filed 7th September 1926. As examples of suitable dispersors the following may be mentioned:—higher fatty acids or sulphonated or other derivatives thereof containing salt-forming groups, for example sulphoricinoleic acid or other sulphated fatty acids, or salts of such acids or derivatives, for instance their alkali or ammonium salts, such acids, derivatives or compounds being generically referred to in U. S. Patent No. 1,618,413 as bodies of oily or fatty characteristics; sulphon-aromatic fatty acids, for example sul-

- pho-benzene stearic acid (Twitchell reagent), sulpho-phenol-stearic acid, sulpho-naphthalene stearic acid, and sulpho-naphthalene ricinoleic acid, or salts of such bodies; carbocyclic compounds containing in their structure one or more salt-forming groups, e. g. naphthenic acids or other carboxylic or sulphonic acids of the cycloparaffins, phenols, sulphonic acids, carboxylic acids, phenols, sulphonic acids, sulphonated naphthalene-formaldehyde condensation products or other derivatives of the benzene, naphthalene or anthracene series or other derivatives of saturated or non-saturated cyclic hydrocarbons containing one or more salt-forming groups, or sodium or other salts of any such compounds; and soluble resin soaps or sodium or other soluble salts or soaps of resin acids.
- 20 As examples of arylides we may mention the anilide, m-nitranilide and p-aniside of  $\beta$ -(2,3) hydroxynaphthoic acid as being particularly useful in connection with the coloring of cellulose acetate, but it will be understood that the invention is not limited thereto but covers the application of any hydroxynaphthoic acid arylide.
- The amines, for application as such or in the diazotized form, may be simple amino bases or aminoazo compounds and in addition to the amino (or diazo) group may have any or a plurality of any other desired substituents, for example nitro, halogen, alkyl, aryl, aralkyl, alkoxy, aryloxy, acylamino, acylamide or thiazol groups. The following are given as examples of suitable diazotizable amino bases but the listing of these examples implies no limitation of the invention thereto:—

*Amino derivatives of benzene*

Aniline.

p-nitraniline.

o-chloraniline.

m-toluidine.

m-nitro-p-toluidine.

4-amino diphenyl.

Benzidine.

Dianisidine.

4-amino-diphenyl methane.

4,4'-diamino-diphenyl methane.

o-anisidine.

p-nitro-o-anisidine.

p-amino-acetanilide.

55 1 - amino-3-p-toluenesulphon amino - benzene.

4-amino-diphenylether.

3-nitro-4-amino-diphenylether.

Dehydrothio-p-toluidine.

60 1-p-amino phenyl-3-methyl-5-pyrazolone.

*Amino derivatives of naphthalene*

$\alpha$ -naphthylamine.

$\beta$ -naphthylamine.

4-nitro-1-naphthylamine.

- 8-chlor-1-naphthylamine.  
1-amino-2-methoxy-naphthalene.  
1,5-naphthylene diamine.  
1-amino-4-acetylamino-naphthalene.  
1 - amino-4-p-toluenesulphonamino - naphthalene. 70

*Amino derivatives of azobenzene*

Aminoazobenzene.

Aminoazotoluene.

4-nitro-4'-aminoazobenzene. 75

4-chlor-2-nitro-4'-aminoazobenzene.

2-nitro-2',4-dimethyl-4'-aminoazobenzene.

4,4' diaminoazobenzene.

2,4-dinitro-3',6'-dimethyl-4'-aminoazoben- 80

zene.  
4-dimethylamino-4'-aminoazobenzene.  
4-methoxy-4'-aminoazobenzene.  
4-phenoxy-2'-methyl-4'-aminoazobenzene.

*Other amino azo compounds*

Aminoazonaphthalene.

Benzene-azo- $\alpha$ -naphthylamine.

2-methoxybenzene-azo- $\alpha$ -naphthylamine.

4-aminobenzene-azo- $\alpha$ -naphthylamine. 90  
4-acetylaminobenzene-azo - $\alpha$  -naphthylamine.

4-nitro-2-methoxy - benzene - azo- $\alpha$  - naphthylamine.

3,5-dinitro-2-hydroxybenzene- azo- $\alpha$ -naphthylamine. 95  
2,4-dinitrobenzene-azo- $\alpha$ -naphthylamine.  
4 - chlornaphthalene-azo - 1-amino-2-methoxynaphthalene.

*Anthraquinone derivatives*

1-aminoanthraquinone.

1-amino-2-methylanthraquinone.

2-aminoanthraquinone.

1-amino-4-hydroxyanthraquinone. 105

1,5-diaminoanthraquinone.

1,8-diaminoanthraquinone.

1-amino-4-acetylaminoanthraquinone.

1-amino-4-bromanthraquinone.

The dispersions of the arylides and the amino compounds or diazo bodies may be applied by any suitable dyeing, printing or stencilling methods. If the amine is to be applied together with the arylide, it may be incorporated in the form of the free base in the dispersion of the arylide. If the amine is to be applied separately it may be applied as a dispersion of the free base or by any other suitable method. 110  
115

The following examples of procedure according to the present invention are intended to be purely illustrative and in no way limitative:—

*Example 1*

To dye 100 kilos of cellulose acetate knit fabric a bright orange shade:—

3 kilos of the m-nitranilide of  $\beta$ -hydroxynaphthoic acid (known commercially as naphthol AS.BS) are reduced to a fine state 130

of subdivision by any suitable means, such for example as precipitation from caustic alkaline solution by acid, or by wet grinding in a so-called colloid mill. The paste thus formed is intimately mixed with 9 kilos of 5 50% Turkey red oil heated to 90° C. diluted suitably with boiling soft water, and passed through a filter cloth into a dyeing machine containing 3000 litres of soft water. The 10 goods are then entered, and the bath raised to 80° C. during 1/2 hour and maintained at that temperature for a further hour. The goods are then washed off, and entered into a 15 3000 litre bath containing 2 1/2 kilos of p-nitraniline diazotized by usual methods, excess of mineral acid being neutralized by addition of the calculated quantity of sodium acetate. The goods are treated for 2 hours at normal temperature, rinsed well, soaped, 20 washed off, and dried or otherwise treated as requisite.

*Example 2*

To dye 100 kilos of cellulose acetate knit fabric a fast navy blue shade:—

25 3 kilos of 4-nitro-2-methoxybenzene-azo- $\alpha$ -naphthylamine, 10% paste, suitably dispersed in 1 kilo 50% Turkey red oil, and 3 kilos m-nitranilide of  $\beta$ -hydroxynaphthoic acid, dispersed as in example 1, are added 30 through a filter cloth to a dyeing machine containing 3000 litres of soft water. The goods are entered into the cold bath, which is raised to 80° C. during 3/4 hour and maintained at that temperature for a further 1 1/2 35 hours. They are now washed off, and entered into a cold bath (30:1 on the goods) containing 2 grams per litre of sodium nitrite and 6 ccs. per litre of hydrochloric acid 28° Tw. After working for 1/2 hour the bath 40 is rendered just alkaline to litmus by cautious addition of soda ash, and the goods worked a further 3/4 hour. After well washing and soaping, the goods are dried, or otherwise treated as requisite.

45 What we claim and desire to secure by Letters Patent is:—

1. In the method of coloring materials comprising organic substitution derivatives of cellulose with hydroxy-naphthoic arylide 50 colors in which the arylide component is applied before diazotization takes place, the step of applying the hydroxy-naphthoic arylide in the free state in the form of a dispersion.

55 2. In the method of coloring materials comprising cellulose acetate with  $\beta$ -hydroxy-naphthoic arylide colors in which the arylide component is applied before diazotization 60 takes place, the step of applying the  $\beta$ -hydroxy-naphthoic arylide in the free state in the form of a dispersion.

3. In coloring materials comprising cellulose acetate with hydroxy-naphthoic arylide 65 colors, applying the hydroxy-naphthoic aryl-

ide in the free state in the form of a dispersion and then applying a diazo solution.

4. In the method of coloring materials comprising cellulose acetate with hydroxy-naphthoic arylide colors in which the arylide 70 component is applied before diazotization takes place, the step of applying the m-nitranilide of  $\beta$ -hydroxynaphthoic acid in the free state in the form of a dispersion.

5. In coloring materials comprising cellulose acetate with hydroxy-naphthoic arylide colors, applying the m-nitranilide of  $\beta$ -hydroxynaphthoic acid in the free state in the form of a dispersion and then applying a diazo solution. 75

6. In coloring materials comprising cellulose acetate, applying a hydroxy-naphthoic arylide in the free state in the form of a dispersion and an amine and subsequently diazotizing. 80

7. In coloring materials comprising cellulose acetate, applying an amine and a hydroxy-naphthoic arylide in the free state together in the form of a dispersion and subsequently diazotizing. 85

8. In coloring materials comprising cellulose acetate, applying  $\beta$ -hydroxy-naphthoic arylide in the free state in the form of a dispersion together with an amine and subsequently diazotizing. 90

9. In coloring materials comprising cellulose acetate, applying the meta-nitranilide of  $\beta$ -hydroxy-naphthoic acid in the free state together with an amine in the form of a dispersion and subsequently diazotizing. 100

In testimony whereof, we have hereunto subscribed our names.

GEORGE HOLLAND ELLIS.  
HENRY CHARLES OLPIN.  
ERIC EATON WALKER.

105

110

115

120

125

130